

## UNITED STATES PATENT OFFICE

2,271,389

## TREATED CASEIN AND PROCESS

John F. Corwin and Robert C. White, Bainbridge,  
N. Y., assignors to The Borden Company, New  
York, N. Y., a corporation of New Jersey

No Drawing. Application January 3, 1940,  
Serial No. 312,302

4 Claims. (CL 106—146)

It is well known that casein dissolves in alkaline solutions, such as solutions of borax, trisodium phosphate, soda ash, potassium carbonate, ammonia, triethanolamine, as well as in the presence of lime. The amounts of these solvents necessary to dissolve a particular casein and the properties of the casein solution when made will depend (among other factors) upon the quality of the particular casein used and this in turn depends upon the manner in which the casein has been prepared from the milk. It is also well known that different commercial caseins vary a great deal in regard to the tendency of the solutions to foam. Such foamy casein solutions are particularly troublesome in most manufacturing processes, for instance, when casein is mixed with clay, satin white or pigments in suspension for use in the paper coating industry. Foamy casein solutions are very objectionable when used as top coatings on paper; for leather finish; in casein paints; in the sizing of cloth and for most purposes where casein solutions are utilized.

Coated paper is used for printing and lithographing in particular. In so coating paper, it is customary to make up what is termed "paper coating color," namely water containing dissolved milk casein and suspended pigments such as clay, satin white, blanc fixe and others (white and/or colored), sometimes also containing dissolved dyestuffs of an alkali resisting nature. When the color has a tendency to foam during the coating operation, bubbles may be formed on the surface of the paper, which break during the drying of the coating, causing pin holes and other imperfections in the coating. Such coated paper does not give a clear and satisfactory surface design, when printed or lithographed.

Many proposals have been made heretofore for a means of preventing the foaming tendency of casein, including the prevention of foaming of paper coating color containing casein. Also to prevent this tendency in casein solutions and mixtures of casein with other substances in general, and so far as we are aware of with only varying degrees of success, small amounts of lard oil mixed with sulphonated oils have been recommended to assist in preventing or limiting this foaming tendency. Other suggestions have been made including the addition of amyl alcohol or pine oil to the casein solution or to paper color or sizing material. Sometimes it has been found necessary to also add small amounts of foam abating agents after a paper color mix has been put into the color box or fountain of the paper coating machine. None of the methods hereto-

fore in common use have been entirely satisfactory.

In our search for a foam abater we have discovered that there are certain chemicals which may be of value as foam abaters or arresters when added to the liquid coating mixture (the "color") and yet which substances applied as a coating to the dried particles of casein prior to dissolving same, do not act in the same manner as regards preventing foam. We have found that certain chemicals are relatively inefficient as foam abaters when added to the prepared coating mixture or to the casein solution, whereas, small amounts of the same chemicals when coated onto the dry casein and the casein thereafter dissolved by the usual methods and tested for foam development, produce remarkably good results, either from the standpoint of largely arresting the tendency to foam in a simple solution of the casein, or in the final mineral-casein-water mixture referred to as "color."

We have in our research made careful tests with a great variety of substances in order to determine their value as foam arresters or foam abaters with casein solutions, by means of coating or spraying onto the dry casein, small amounts of various substances for this purpose. During this series of tests we have found for example that when a relatively small percentage of tributyl phosphate is mixed into a casein solution or into a paper "color," it is fairly satisfactory for reducing tendency to foam, yet this same tributyl phosphate when put onto the dry casein (e. g. as a spray), and the casein thereafter dissolved in the usual way, does not to the same extent stop or arrest the foaming tendency. In a number of other instances this peculiar condition has been found with various chemicals; and with certain other chemicals, the reverse condition exists.

As the basis of the present invention, we have found that it is possible to very greatly reduce the tendency of paper coating mixtures containing casein to foam, by applying to the solid, dry casein, which is to be dissolved and used in paper coating mixtures, a small amount of tributyl citrate. This citrate should be applied to the solid casein while the latter is preferably in the air-dry condition, before the said casein is dissolved in alkali. In fact when an equal amount of the tributyl citrate is added to a paper coating color already prepared, or to other casein solutions, it does not give such good results, i. e. it does not reduce the tendency to foam to such an extent as when applied to the solid casein, before dis-

solving. Thus, very useful results have been produced by spraying the tributyl citrate upon the dry casein (or in any other manner coating the casein particles with the small amount of tributyl citrate), and subsequently dissolving the casein in an alkali solution, and incorporating the pigments, etc. The best amount of the tributyl citrate to be used with a particular casein, to give the most satisfactory results, should first be determined as for that particular lot of casein. In using high grade caseins, we have sometimes found small amounts such as 0.2% to be satisfactory, although in some cases where the foaming tendency of the casein is high, we prefer to use much larger amounts such as 1%. Based on our experimentation to date, we believe that not more than 5% of the tributyl citrate would be necessary in any case. After adding the citrate, the casein can be dissolved at once, or after storage, shipping, etc.

In order to more fully explain our invention we give herewith by way of illustration, several examples of the utilization of the discoveries leading up to this process, although we do not limit ourselves in any way to the examples cited.

#### EXAMPLE 1

Into a suitable mixer such as the usual spiral mixer containing the proper spiral agitator, we placed 400 parts of ordinary commercial casein which had been ground, for example, to all pass through a standard 24 mesh wire screen. The spiral in the mixer, by any convenient means, was made to revolve at a fairly rapid speed and thereafter we sprayed 1 part (=0.25%) of commercial tributyl citrate onto the casein while being agitated in the spiral mixer. Thereafter, operation of the mixer was continued for about 5 minutes, the material then removed from the mixer and tested for foaming tendency as follows:

100 gms. of the tributyl citrate treated casein was added to 500 gms. of cold water, mixed to wet the particles and allowed to stand for about 10 to 15 minutes. Thereafter we added 7 gms. of commercial 26° ammonia, the liquid mass, mixed thoroughly and thereafter the receptacle holding the mixture was placed in a water bath and heated, while stirring slowly, to about 140° F. When the casein was completely dissolved we slowly added a further 500 gms. of cold water to this solution, stirring it thoroughly to obtain a uniform solution which was then cooled to 75° F. We then made a test to determine the relative foaming tendency of this treated casein by the following method:

Into a one-quart capacity cylindrical glass jar there was placed 400 cc. of the casein solution above referred to and the height of the liquid was marked on the jar. One egg-beater mounted on a Sunbeam Mix-Master mixer was placed in the solution. The beater was started, the beater running 640 R. P. M. and the beating was continued for exactly 6 minutes (by a stop-watch). Then the beating was discontinued and the height of the liquid plus the foam developed was quickly measured. This by subtraction showed the "height of foam" developed from the top of the original liquid in the jar to the top of the foam layer. This height of foam developed applies to the particular casein used in this example, modified by the tributyl citrate.

After having measured the height of foam, the solution in the jar was allowed to rest undisturbed for another 5 minute period and a second

measurement taken to indicate the degree of speed with which the developed foam receded or broke down. Thereafter the solution was allowed to rest for a sufficient length of time to allow the foam which was developed during this test to entirely recede.

10 A control test, duplicating and paralleling in every particular the above referred to example, was made with another sample from the same lot of casein, same method of dissolving and testing but without the addition of any tributyl citrate.

15 The results of both these tests are recorded in Table No. I, below.

#### EXAMPLE 2

20 400 parts of casein, 3 parts of tributyl citrate, mixed and prepared exactly as described in Example No. 1. The casein was from the same lot as used in Example 1. A 100 gram sample of this mixture was then dissolved and tested for foaming tendency in the exact manner described under Example No. 1.

25 The results of these tests are recorded under Table I.

30 Other tests with other types of casein known to possess much greater foaming tendencies than the casein used in Examples 1 and 2, were also treated with various amounts of tributyl citrate by means of spraying or "oiling" the ground dry casein, one particular casein being one known to be extremely difficult to use in commercial operations, from the standpoint of dissolving or preparing the solution because of its great tendency to foam (even foaming over the mixing kettles while the solution is being prepared, unless extra care is used in its preparation). Such a casein was used in Examples 3 and 4.

#### EXAMPLE 3

35 400 parts of a casein (known to be excessively foamy), 3 parts of tributyl citrate. Procedure for preparation was exactly the same as described under Example 1. Thereafter a sample of 100 grams of this mixture was dissolved and the "height foam" determined as described under Example 1. The results of these tests appear in Table I.

#### EXAMPLE 4

40 400 parts of this same casein, 1 part of tributyl citrate. Procedure for preparation exactly the same as described under Example 1. Thereafter a sample of 100 parts of this mixture was dissolved and tested for "height of foam" as described under Example 1. The results of these tests appear in Table I.

45 A control (without the citrate added) on the casein used in Examples 3 and 4, was treated and tested in the same way.

#### EXAMPLE 5

50 400 parts of commercial sodium caseinate ground to a fineness so that all will pass through a 24 mesh screen. To this was added 4 parts of tributyl citrate following the method as described in Example 1. Thereafter, 100 grams of the treated sodium caseinate was added to 500 cc. of cold water, mixed to wet the particles and immediately heated (because sodium caseinate is soluble in water without the addition of other solvents) to about 140° F. After the casein was dissolved we added 500 cc. of cold water and stirred the mixture until it was in a uniform

consistency. Thereafter this solution was tested for its "height of foam", as per the method described under Example 1 and the results are recorded in Table I.

A sample of this same sodium caseinate without tributyl citrate was similarly treated, as a control, and the results are shown in Table I.

Table I

| Example               | Percent tributyl citrate | Foam after 6 minutes beating | Foam after 5 minutes rest | Foam all broken down | Minutes |
|-----------------------|--------------------------|------------------------------|---------------------------|----------------------|---------|
| Control on 1 and 2.   | 0                        | Inches                       | Inches                    |                      | 60      |
|                       | 0.25                     | 1                            | 0.375                     |                      | 10      |
|                       | 0.75                     | 0.250                        | 0.0625                    |                      | 7       |
| Control on 3 and 4.   | 0                        | 1.500                        | 0.125                     |                      | 25      |
|                       | 0.75                     | 0.875                        | None                      |                      | 4       |
|                       | 0.25                     | 1.125                        | 0.0313                    |                      | 8       |
| Control on Example 5. | 0                        | 1.812                        | 1.812                     |                      | 150     |
|                       | 1                        | 1.125                        | 0.750                     |                      | 20      |

Other tests were made by preparing a complete color mixture and thereafter making a foam test with this color mixture by the usual well established method (described below) to determine the "foam index" in paper coating color mixtures. In one of these tests the material prepared under Example 3 was used (with pigments).

In another test the same casein without treatment with tributyl citrate was employed.

The results of these tests are indicated in Table II.

The method used for preparing and making the paper color foam index test was as follows:

A casein solution was made up at a concentration of 1 part of the particular casein to 5 parts of water, using ammonia as given in Example 3 as the solvent for the casein. Other solvents could be used as long as the same solvent is used in comparative tests.

A clay slip was made up by mixing 1 part of clay with 1 part of water to a smooth paste. To 200 parts of the clay slip were added 66 parts of the casein solution which is equivalent to 11 parts dry casein. This was mixed until smooth and strained through a wire screen to insure complete uniformity (a 100 mesh screen was used in the present tests).

The weight of 100 cc. of the clay-casein mix was determined. 200 grams of the mix were weighed into a 400 cc. low form beaker and stirred for 2 minutes at 2700 R. P. M. with a horizontal flat stirring disc 1 inch in diameter and  $\frac{1}{8}$  inch thick, the disc being immersed in the mix so that the top of it is  $\frac{3}{4}$  inch below the surface of the liquid. At the end of two minutes stirring, the mix was allowed to stand for one minute. Immediately, thereafter, the weight of 100 cc. of the so treated mixture was determined. The loss in weight as compared with the weight of 100 cc. mentioned above, is termed the "foam index."

Table II

|                                                  | Foam index |
|--------------------------------------------------|------------|
| Color mix (casein not treated)                   | 48.5       |
| Color mix (casein treated with tributyl citrate) | 0          |

As will be noted from the results indicated in Table I and Table II, we obtain a very marked decrease in the foaming tendency in the casein solutions themselves, and in the paper "color" made from the casein, by means of the addition

of these relatively small amounts of tributyl citrate. We do not wish to limit our invention to any definite amount of tributyl citrate to be added to the dry casein but we have thus far found that not over 1% of tributyl citrate seems to be sufficient on any of the caseins we have examined. We believe that quantities below 5% will be sufficient in all cases.

All of the above specific disclosure, including the above examples and the above tables, refers to the treatment of "milk casein."

The invention is also applicable with satisfactory results to the treatment of "vegetable casein," which may be, to some extent, considered as a substitute for "milk casein" in the paper coating art. This material also often shows a troublesome foaming tendency.

Various tests were made by treating isolated soybean protein (which material is referred to in the literature and in commerce, as "vegetable casein" or "soya casein"), with tributyl citrate by the process described herein, in order to reduce the foaming tendency of products of this nature, namely, isolated vegetable protein. Tests were made as follows: An isolated soybean protein (which in many of its properties is similar to milk casein) was purchased on the market. This is of a type that is commercially offered to the trade regularly.

#### EXAMPLE 6

Into a suitable mixer such as the usual mixer containing the proper spiral agitator, we placed 400 parts of dry ground soy-bean isolated protein (also sometimes called "soya casein"). The spiral mixer, by any convenient means, was made to revolve at a fairly rapid speed and thereafter we sprayed 1 part (0.25%) of commercial tributyl citrate onto the isolated protein while being agitated in the spiral mixer. Thereafter the mixing was continued for about 5 minutes, the material then removed from the mixer and tested for foaming tendencies. The procedure for dissolving and testing the resulting mixture for foaming tendency was the same as that described under Example 1, with the exception that a little more ammonia was used as the solvent, namely 10 grams of ammonia in this case instead of 7 grams as used in Example 1.

#### EXAMPLE 7

The same procedure was followed as in Example 6 with the exception that we used 2 parts (0.50%) of commercial tributyl citrate.

#### EXAMPLE 8

Same as Example 6, with the exception that we used 3 parts (0.75%) of commercial tributyl citrate.

#### EXAMPLE 9

The same as Example 6, with the exception that we used 4 parts (1%) of commercial tributyl citrate.

The resulting solutions of the treated isolated soya protein (made in Examples 6 to 9) were tested for foaming tendencies in the same manner as described under Example 1 and for purpose of control, an untreated sample of the same isolated soya protein (without the citrate added) was dissolved in the same manner as described under Example 1. The results obtained in Examples 6 to 9 inclusive plus the control test are indicated in Table III.

Table III

| Example | Percent tributyl citrate | Foam after 6 minutes beating | Foam after 5 minutes rest | Foam all broken down |
|---------|--------------------------|------------------------------|---------------------------|----------------------|
| Control | 0                        | Inches                       | Inches                    | Minutes              |
| 6       | 0.25                     | 2.063                        | 1.875                     | 40                   |
| 7       | 0.50                     | 0.938                        | 0.50                      | 9                    |
| 8       | 0.75                     | 0.875                        | No foam                   | No foam              |
| 9       | 1                        | No foam                      | No foam                   | No foam              |

In some cases (in which the most extreme smoothness is not needed, as in coating wall paper), instead of the "isolated vegetable protein," we can use a solvent extracted seed meal, e. g. a solvent extracted soybean press cake which has been pressed cold or at a relatively low temperature. This material is ground to an extremely fine condition, and can be used with or without milk casein or isolated vegetable casein, being treated with tributyl citrate and thereafter dissolved in a mildly alkaline solution, with or without pigments and/or dyes, and then used for coating paper.

It is to be understood that after applying the tributyl citrate to the casein, the latter can be stored for a long time, or can be shipped, and/or compounded with any of the materials with which casein is usually compounded, before being dissolved, and the "non-foaming" property of the so treated casein will persist. Thus we may treat the casein at the factory and ship this to a paper-coating mill to there be dissolved as wanted.

The term "casein," as used in the appended claims, is intended to include milk casein and isolated vegetable proteins "vegetable casein" and the finely ground solvent-extracted seed meal and also caseinates in general, such as sodium caseinate, ammonium caseinate, magnesium caseinate, etc., which last three are compounds of milk casein with a small amount of soda, ammonia or magnesia. Mixtures of such materials are also included.

The casein is preferably, at the beginning of the step of oiling with the citrate, in the usual "air dry" condition, and the citrate can be used alone or mixed with solvents or diluents (e. g. alcohol, etc.), which also are non-aqueous liquids, but do not have to be completely anhydrous. The term "non-aqueous liquids" is used in the appended claims to distinguish from liquids which consist largely of water.

The tributyl citrate, given in the above examples and specific disclosure, is an alkyl citrate, and tributyl citrate is generally about the most satisfactory alkyl citrate to employ. We do not desire to restrict all of the claims to the butyl compound, nor to the tri-alkyl compound, because alkyl citrate broadly, applied to the casein while the latter is in the solid state will be (to some extent at least) effective.

We claim:

1. A process of producing casein solutions of reduced foaming tendency which comprises applying to solid casein, a small amount of tributyl citrate, the amount of the latter being not substantially above 5%, based on the amount of said casein, and thereafter dissolving the casein in an aqueous solvent.

2. A process which comprises agitating a mass of comminuted solid casein while spraying a substantially non-aqueous liquid material containing tributyl citrate upon said casein, the amount of said citrate being not substantially more than 5%, based on the casein, and thereafter dissolving the so-treated casein in an aqueous alkaline liquid, whereby a casein solution is produced having not more than a low foaming tendency.

3. Solid casein carrying intimately incorporated therewith, an amount of tributyl citrate which is not substantially in excess of 5%, based on the weight of the casein.

4. Solid casein wetted with a fraction of one per cent of tributyl citrate.

JOHN F. CORWIN.  
ROBERT C. WHITE.